

# United States Patent Office

2,735,790

Patented Feb. 21, 1956

1

2,735,790

## COMPOSITION AND METHOD FOR IMPARTING SOFTNESS AND ANTI-STATIC PROPERTIES TO ACRYLONITRILE FIBERS

Calvin J. Waikus, Decatur, Ala., assignor to The Chemstrand Corporation, Decatur, Ala., a corporation of Delaware

No Drawing. Application October 20, 1954,  
Serial No. 463,589

9 Claims. (Cl. 117—138.8)

This invention relates to the treatment of shaped articles, and relates more particularly to an improved process for imparting antistatic, lubricity, softness and other desirable properties to articles comprising acrylonitrile polymers, to the articles resulting from such process, and to compositions employed therein.

Acrylonitrile polymers constitute a class of material which develop, or tend to develop, an electrostatic charge upon their surfaces when fibers or other articles made therefrom are subjected to friction during their production and during processing or fabrication of the fibers into fabrics or other articles, as well as during the use of the finished article. Before fibers of acrylonitrile polymers are spun into yarns it is necessary to modify the electrical qualities so that the fibers will generate a minimum amount of electricity during carding, combing, spinning, and like operations where the fibers are rubbed in constant frictional contact. The presence of static electricity on the fibers creates a severe problem, because it not only results in sticking of the fibers to the machinery, but also tends to cause the fibers to repel each other during such operations as carding and drawing so that it is difficult or impossible to spin a coherent, compact yarn from them.

Another problem of major importance encountered with filaments and fibers of acrylonitrile polymers is to so lubricate or soften the yarn that it will have the correct frictional characteristics, or drag, and the required flexibility for the specific purpose in view. In the handling of continuous filament yarn, for example, it is necessary to condition the material to reduce the tendency toward breakage of individual filaments when the yarn is subjected to mechanical strains such as are involved in passage of the yarn over guides, rolls, and other parts of the yarn-producing mechanism and in twisting, winding, reeling and similar operations. In the case of yarns intended for use on commercial knitting machinery, it is particularly important that the yarn be soft and pliable in order that it may conform to the contour of the needles and give a closely knit fabric free from cuts, pinholes, stitch distortion, laddering, misplaits and other common defects.

Although shaped articles of acrylonitrile polymers generally may be treated in accordance with this invention for modification of their properties, the process is of special advantage in the treatment of fibers to render them more amenable to textile processing, and will be described in detail in connection with such use.

The fibers to be conditioned in accordance with this invention may be formed of polyacrylonitrile, or copolymers containing at least about 80 percent acrylonitrile and up to about 20 percent of other monomers copolymerizable therewith. Examples of suitable monomers which may be copolymerized with acrylonitrile to form the fibers which can be treated in accordance with this invention are acids such as acrylic, haloacrylic, and methacrylic acids; esters such as methyl, butyl, octyl, methoxymethyl, and chloroethyl methacrylates and the corresponding esters of acrylic and haloacrylic acids; meth-

2

acrylonitrile; vinyl and vinylidene halides such as vinyl chloride, vinyl fluoride, vinylidene chloride, 1-fluoro-1-chloroethylene; vinyl carboxylates such as vinyl acetate, vinyl chloroacetate, vinyl propionate, and vinyl stearate; 5 N-vinylimides such as N-vinylphthalimide, and N-vinylsuccinimide; N-vinyl lactams such as N-vinylcaprolactam and N-vinylbutyrolactam; aryl compounds such as styrene and vinyl naphthalene; and other compounds such as methyl vinyl ketone, methyl fumarate, methyl vinylsulfone, fumaronitrile, maleic anhydride, the vinylpyridines such as 2-vinylpyridine, 3-vinylpyridine, and 4-vinylpyridine, the vinyl-substituted alkyl pyridines such as 4-ethyl-2-vinylpyridine, 5-ethyl-2-vinylpyridine, and 2-methyl-5-vinylpyridine; the isomeric vinylpyrazines, the various isomeric vinylquinolines, the vinylimidazoles and the vinylbenzoxazoles.

The fibers or filaments may also be formed from a mixture of two or more of the fiber or film-forming materials. For example, the fibers, films, or other shaped articles to be rendered conditioned may be formed from or comprise a blend of a base acrylonitrile polymer with other polymeric materials which modify the base polymer in various respects, as by imparting dye-receptivity thereto, increasing the flame-resistance thereof, or increasing the hydrophylic properties of the polymer, etc. Suitable polymeric materials for blending with the base polymer, which may be polyacrylonitrile or binary or ternary copolymers of acrylonitrile with the copolymerizable substances mentioned above are those polymeric materials which are soluble in the same solvent as the base polymer and which, when mixed with the base polymer in an amount of from about 2 to 50 percent on the weight of the blend, result in a blend which forms a solution of at least 5 percent concentration in the solvent, 15 which solution can be formed into fibers by conventional procedures. Suitable solvents are dimethyl formamide, dimethyl acetamide, gamma-butyrolactone, ethylene carbonate, and others disclosed in such patents as U. S. Nos. 2,404,712 to 2,404,727; 2,498,605; 2,522,445; 2,487,839; 2,606,168 and 2,496,267.

As an illustration, the blend may comprise a base polymer such as a copolymer containing at least 80 percent by weight of acrylonitrile and up to 20 percent by weight of another monoethylenically unsaturated monomer as recited above with from 2 to 50 percent by weight of a copolymer containing from 10 to 70 percent of acrylonitrile and from 30 to 90 percent of another monoethylenically unsaturated material which is different from the comonomer in the base polymer, for example, from 30 to 90 percent of a vinyl-substituted heterocyclic tertiary amine, and preferably a vinylpyridine.

In accordance with the process of this invention, the shaped articles comprising acrylonitrile polymers, copolymers and blends are conditioned by treating them with an aqueous emulsion, the solids content of which comprises from about 20 to 50 percent by weight of a non-ionic surface active ester, from 15 to 35 percent of a non-ionic surface active polyether, from 10 to 40 percent of a cationic surface active quaternary ammonium compound and from 5 to 25 percent of a substituted carbamyl derivative, all of which are more particularly defined hereinafter. The esters comprising an essential part of the agents of this invention are preferably long chain fatty acid partial esters of polyhydric alcohols or their anhydrides, such as sorbitan monopalmitate and sorbitan monolaurate. The non-ionic surface active agents, referred to herein generally as polyethers, can be prepared by condensing a water-insoluble hydroxy-fatty acid, or esters of such acid, or mixture of such acid or ester, with from 150 to 250 parts of ethylene oxide.

Among the polyhydric alcohols or anhydrides from which the partial esters may be made are those having

from 2 to 8 carbon atoms, such as mannitol, sorbitol, glucose, erythritol, pentaerythritol, glycols such as ethylene glycol, triethylene glycol, propylene glycol, diethylene glycol, tetraethylene glycol, etc. Various saturated and unsaturated aliphatic acids may be reacted with the polyhydric alcohols in making the partial esters. A preferred group of partial esters are those containing a single ester linkage. However, partial esters containing more than one ester linkage may be used.

The acid used in making the partial esters may be saturated or unsaturated aliphatic acids containing from 10 to 20 carbon atoms. Preferred acids are those which are saturated or contain only one olefinic group. Examples of such acids include mono-olefinic unsaturated aliphatic acids such as 7-hexadecenoic acid, 10-undecenoic acid, 13-docosenoic acid and 9-octadecenoic acid; substituted olefinic acids, for example, such hydroxy olefinic acids as 16-hydroxy-7-hexadecenoic acid and 12-hydroxy-9-octadecenoic acid; halogenated unsaturated acids, for example, monochloro-9-octadecenoic acid, monochloro-12-hydroxy-9-octadecenoic acid, and halogenated acids derived by dehydration of castor oil acids followed by chlorination; saturated fatty acids such as decanoic acid, undecanoic acid, dodecanoic acid, tridecanoic acid, tetradecanoic acid, pentadecanoic acid, hexadecanoic acid, heptadecanoic acid, octadecanoic acid, and nonadecanoic acid. These saturated acids may also have straight or branched chains, or substituted chains, and may be substituted, for example, with chlorine or other halogen atoms, as for example, monochlorooctadecanoic acid, and the like.

Specific partial esters suitable for use in this invention include glyceryl monohexadecanoate, glyceryl monododecanoate, glyceryl mono-9-octadecanoate, glyceryl mono-12-hydroxy-octadecanoate, sorbitan monododecanoate, propylene glycol mono-octadecanoate, ethylene glycol mono-octadecanoate, diethylene glycol mono-octadecanoate, and sorbitan mono-octadecanoate.

Examples of hydroxy-fatty acids which can be used as such, or in the form of partial esters with the polyhydric alcohols set forth above, for condensation with ethylene oxide to form the ether portion of the compositions of this invention, include both saturated and unsaturated hydroxy acids such as 12-hydroxy-octadecanoic acid, 12-hydroxy-dodecanoic acid, 16-hydroxy-hexadecanoic acid, 11-hydroxy-hexadecanoic acid, 10-hydroxy-octadecanoic acid, 3,12-dihydroxy-palmitic acid, 9,10,16-hydroxy-hexadecanoic acid, 9,10,12,13-hydroxy-octadecanoic acid, 16-hydroxy-7-hexadecanoic acid, 12-hydroxy-9-octadecanoic acid.

The cationic surface active agents used in this invention are the quaternary ammonium compounds having the formula:



wherein R represents an alkyl radical having less than 5 carbon atoms, R' represents an alkyl radical having less than 5 carbon atoms, and R'' represents an alkyl radical having more than 10 carbon atoms.

The substituted carbamyl derivatives which are an essential ingredient of the compositions of this invention are those having the general formula:



In the formula R<sub>1</sub> and R<sub>6</sub> may be the same or different and are preferably saturated aliphatic chains containing at least 6 carbon atoms; R<sub>2</sub>, R<sub>3</sub>, R<sub>4</sub> and R<sub>5</sub> each represent hydrogen, or a simple alkyl or hydroxyalkyl radical of less than 5 carbons and R<sub>2</sub> and R<sub>4</sub> may further represent an acid amide chain derived from an acid and a polyamine; D<sub>1</sub> and D<sub>2</sub> represent oxygen, sulfur, or an imido group; the number of such groups being as g ranges from 0 to 3; g represents a whole number from 0 to 3; A represents either oxygen, sulfur, an amino group, or a simple alkyl or alkylol-substituted amino group of less than five carbons (such as NC<sub>2</sub>H<sub>4</sub>OH or NC<sub>2</sub>H<sub>5</sub>); f and j represent whole numbers from 1 to 6 preferably from 1 to 3; e and k represent whole numbers from 0 to 6, preferably from 0 to 3; m and t represent whole numbers from 1 to 6, preferably not over 2, and one of the hydrogens in each dimethylene group may be substituted by a methyl group; B represents the hydrogen of an acid or alkyl group; and X represents a negative radical such as an acyl radical or a halogen.

Substances embraced by the formula given can be obtained by condensing a saturated acid, acid ester, or acid halide with an aliphatic polyamine, reacting the condensate with a carbamyl compound, and then converting the substituted carbamyl derivatives thus obtained to its corresponding acid salt or alkylated product.

Acids which may be condensed with polyamines to obtain the condensates are the saturated acids containing at least 6 carbon atoms, such as lauric, stearic, palm oil acids, etc.

The acids may be condensed with any of the aliphatic polyamines, such as ethylene diamine, diethylene triamine, triethylene tetramine, tetraethylene pentamine, hexamethylene diamine, hydroxyethyl ethylene diamine, ethyl ethylene diamine, 2,2-dimethyl-1,3-diaminopropane, 1,3-diaminoisopropanol, beta, beta-diamino-diethyl ether and beta-beta-diamino diethyl thioether.

The carbamyl compounds which are reacted with the acid-amino condensate include urea, thiourea, guanidines, biurets, guanylureas, and diguanidines.

For the purpose of this invention, the substituted carbamyl derivatives must be converted to their acid salts or alkylated products. The acid salts are obtained by reacting the carbamyl derivatives with an acid, for example, with acetic, lactic, boric, oxalic, benzoic, salicylic, furoic, citric, tartaric; formic, phthalic, succinic, or alkyl naphthalene sulfonic acids. The alkylated products are obtained by after-treating the substituted carbonyl derivative with an alkylating agent such as ethyl chloride, benzyl chloride, ethylene oxide, ethylene chlorhydrin, or dimethyl sulfate.

The acid-amino condensates can be prepared by heating equimolar quantities of the selected saturated acid and of the polyamine at temperatures from 130 to 200° C. until the reaction is complete as shown by the loss of one molecule of water. The mix is then cooled to 180° C. and one half mol or more of urea or other carbonyl compound is added. Ammonia is rapidly liberated as the urea becomes substituted, the temperature being maintained at between 170 and 200° C. The product thus obtained is then reacted with the appropriate acid or with an alkylating agent to produce the compounds designated by the structural formula.

The compositions of this invention are preferably used as aqueous dispersions, and from 1 to 5 percent solids in such dispersions has been found to give most satisfactory results. The compositions can be applied to the fibers in any suitable manner, as by dipping or immersing the fiber in the medium, by spraying or dripping, by means of a wick or roller, etc.

In the conventional practice, fibers and other articles comprising the acrylonitrile polymers, copolymers and blends, are stretched in the course of their production, for orientation of the molecules and improvement in their tenacity. If the fibers are steam-stretched, after washing thereof to partially or completely remove the spinning sol-

vent, the anti-static medium is applied to the fibers after washing. For some purposes, the heat-stretching for orientation may be dispensed with. If the fibers are not stretched in a steam atmosphere, the finishing medium may be applied to them any time subsequent to their withdrawal from the spinning zone and washing thereof for removal of the spinning solvent and drying. Thus it may be applied to continuous filaments or to discontinuous fibers obtained by cutting or otherwise disrupting the filaments, and before or after crimping of the filaments or fibers. However, in the preferred embodiment of this invention, the finishing composition set forth above is applied to a running tow or bundle of fibers which may occur in the tow or bundle in continuous or discontinuous form.

The application of the compositions of this invention are illustrated in the following examples:

*Example I*

An aqueous dispersion was prepared containing 2 percent solids, of which 48 percent by weight was sorbitan monopalmitate, 32 percent was the product obtained by condensing castor oil with 200 mole equivalents of ethylene oxide, 10 percent was N-cetyl, N-ethyl morpholinium ethosulfate and 10 percent was  $\alpha, \beta$ -dihydroxyethyl- $\alpha', \beta'$ -di( $\beta$ -stearamidoethyl) urea acetate. This composition was applied to a tow obtained by spinning a blend of a first copolymer containing 97 percent acrylonitrile and 3 percent vinyl acetate with a second copolymer containing 50 percent acrylonitrile and 50 percent 2-methyl-5-vinylpyridine. The overall 2-methyl-5-vinylpyridine content of the blend was 6 percent. Application was accomplished by immersing the tow in the dispersion. Analysis of the treated tow showed from 0.5 to 1.5 percent of the finish present, based on the tow weight. The resulting cut staple was found to be more open, softer and better lubricated than the same staple treated in a like manner with a dispersion containing 2 percent solids of which 54 percent was sorbitan monopalmitate, 36 percent was the castor oil-ethylene oxide condensate, and 10 percent was N-cetyl, N-ethyl morpholinium ethosulfate.

*Example II*

An aqueous dispersion was prepared containing 1.5 percent solids, of which 42 percent by weight was sorbitan monopalmitate, 28 percent was the product obtained by condensing castor oil with 200 mole equivalents of ethylene oxide, 20 percent was N-cetyl, N-ethyl morpholinium ethosulfate and 10 percent was  $\alpha, \beta$ -dihydroxyethyl- $\alpha', \beta'$ -di( $\beta$ -stearamidoethyl) urea acetate. This composition was applied in the same manner as described in Example I to a tow of the same blended acrylic polymer fiber. The resulting cut staple was found to be more open, softer, and better lubricated, and exhibited a considerably less tendency toward the development of static electricity during textile processing, such as carding and drawing of the staple fibers, than did the same staple treated in a like manner with a dispersion containing 1.5 percent solids of which 54 percent was sorbitan monopalmitate, 36 percent was the castor oil-ethylene oxide condensate, and 10 percent was N-cetyl, N-ethyl morpholinium ethosulfate.

*Example III*

There was applied to a tow of the same blended acrylic polymer fiber in same manner as above an aqueous composition containing 1.5 percent solids, of which 36 percent by weight was sorbitan monopalmitate, 24 percent was the castor oil-ethylene oxide condensate product, 20 percent was N-cetyl, N-ethyl morpholinium ethosulfate and 20 percent was  $\alpha, \beta$ -dihydroxyethyl- $\alpha', \beta'$ -di( $\beta$ -stearamidoethyl) urea acetate. Again the improvement in openness, softness, and lubricity of the cut staple was evident over the same staple treated with the three-component composition.

I claim:

1. As a new composition of matter, a mixture comprising from 20 percent to 50 percent by weight of a non-ionic surface active partial ester of a polyhydric alcohol and an aliphatic carboxylic acid, said alcohol having from two to 8 carbon atoms, from 15 percent to 35 percent of a non-ionic surface active polyether prepared by condensing from 150 to 250 parts of ethylene oxide with a member selected from the group consisting of water-insoluble hydroxy-fatty acids, esters of such acids, and mixtures of such acids and esters, from 10 percent to 40 percent of a cationic surface active quaternary ammonium compound having the formula:



wherein R represents an alkyl radical having less than 5 carbon atoms, R' represents an alkyl radical having less than 5 carbon atoms, and R'' represents an alkyl radical having more than 10 carbon atoms, and from 5 percent to 25 percent of a substituted carbamyl compound having the formula:



wherein R<sub>1</sub> and R<sub>6</sub> are selected from the group consisting of saturated alkyl radicals containing at least 6 carbons; R<sub>2</sub>, R<sub>3</sub>, R<sub>4</sub>, and R<sub>5</sub> are selected from the group consisting of hydrogen, alkyl, and hydroxylalkyl radicals containing less than 5 carbons and in which R<sub>3</sub> and R<sub>4</sub> may further represent an acid amide chain derived from an acid and a polyamine; D<sub>1</sub> and D<sub>2</sub> are selected from the group consisting of oxygen, sulfur, and imido groups, the number of such groups being as g ranges from 0 to 3; g is an integer from 0 to 3; A is selected from the group consisting of oxygen, sulfur, amino groups, alkyl-substituted amino groups containing less than 5 carbons, and alkylol substituted amino groups containing less than 5 carbons; f and j are integers from 1 to 6; e and k are integers from 0 to 6; m and i are integers from 1 to 6; and X is a negative radical selected from the group consisting of acyl and halogen.

45

50

55

60

65

70

75

2. As a new composition of matter, an aqueous dispersion containing from one to 5 percent solids, said solids comprising from 20 percent to 50 percent by weight of a non-ionic surface active partial ester of a polyhydric alcohol and an aliphatic carboxylic acid, said alcohol having from two to 8 carbon atoms, from 15 percent to 35 percent of a non-ionic surface active polyether prepared by condensing from 150 to 250 parts of ethylene oxide with a member selected from the group consisting of water-insoluble hydroxy-fatty acids, esters of such acids, and mixtures of such acids and esters, from 10 percent to 40 percent of a cationic surface active quaternary ammonium compound having the formula:



wherein R represents an alkyl radical having less than 5 carbon atoms, R' represents an alkyl radical having less than 5 carbon atoms, and R'' represents an alkyl

radical having more than 10 carbon atoms, and from 5 percent to 25 percent of a substituted carbamyl compound having the formula:



wherein R<sub>1</sub> and R<sub>6</sub> are selected from the group consisting of saturated alkyl radicals containing at least 6 carbons; R<sub>2</sub>, R<sub>3</sub>, R<sub>4</sub> and R<sub>5</sub> are selected from the group consisting of hydrogen, alkyl, and hydroxyalkyl radicals containing less than 5 carbons and in which R<sub>3</sub> and R<sub>4</sub> may further represent an acid amide chain derived from an acid and a polyamine; D<sub>1</sub> and D<sub>2</sub> are selected from the group consisting of oxygen, sulfur, and imido groups, the number of such groups being as g ranges from 0 to 3; g is an integer from 0 to 3; A is selected from the group consisting of oxygen, sulfur, amino groups, alkyl-substituted amino groups containing less than 5 carbons, and alkylol substituted amino groups containing less than 5 carbons; f and j are integers from 1 to 6; e and k are integers from 0 to 6; m and t are integers from 1 to 6; and X is a negative radical selected from the group consisting of acyl and halogen.

3. As a new composition of matter, an aqueous dispersion containing from one to 5 percent solids, said solids comprising from 20 percent to 50 percent by weight of sorbitan monopalmitate, from 15 percent to 35 percent of castor oil condensed with from 150 to 250 parts of ethylene oxide, from 10 percent to 40 percent of N-cetyl, N-ethyl morpholinium ethosulfate, and from 5 percent to 25 percent of  $\alpha$ ,  $\beta$ -dihydroxyethyl- $\alpha'$ ,  $\beta'$ -di( $\beta$ -stearamidoethyl) urea acetate.

4. The composition of claim 3 wherein the solids content is about one and one-half percent.

5. The method of imparting lubricity, softness and anti-static properties to shaped articles comprising an acrylonitrile polymer containing by weight in the molecule at least 80 percent of acrylonitrile which comprises applying to the article an aqueous dispersion containing from one to 5 percent solids, said solids comprising from 20 percent to 50 percent by weight of a non-ionic surface active partial ester of a polyhydric alcohol and an aliphatic carboxylic acid, said alcohol having from two to 8 carbon atoms, from 15 percent to 35 percent of a non-ionic surface active polyether prepared by condensing from 150 to 250 parts of ethylene oxide with a member selected from the group consisting of water-insoluble hydroxy-fatty acids, esters of such acids, and esters, from 10 percent to 40 percent of a cationic surface active quaternary ammonium compound having the formula:



wherein R represents an alkyl radical having less than 5 carbon atoms, R' represents an alkyl radical having less than 5 carbon atoms, and R'' represents an alkyl radical having more than 10 carbon atoms, and from 5

percent to 25 percent of a substituted carbamyl compound having the formula:



15 wherein R<sub>1</sub> and R<sub>6</sub> are selected from the group consisting of saturated alkyl radicals containing at least 6 carbons; R<sub>2</sub>, R<sub>3</sub>, R<sub>4</sub>, and R<sub>5</sub> are selected from the group consisting of hydrogen, alkyl and hydroxyalkyl radicals containing less than 5 carbons and in which R<sub>3</sub> and R<sub>4</sub> may further represent an acid amide chain derived from an acid and a polyamine; D<sub>1</sub> and D<sub>2</sub> are selected from the group consisting of oxygen, sulfur, and imido groups, the number of such groups being as g ranges from 0 to 3; g is an integer from 0 to 3; A is selected from the group consisting of oxygen, sulfur, amino groups, alkyl-substituted amino groups containing less than 5 carbons, and alkylol substituted amino groups containing less than 5 carbons; f and j are integers from 1 to 6; e and k are integers from 0 to 6; m and t are integers from 1 to 6; and X is a negative radical selected from the group consisting of acyl and halogen.

6. The method of imparting lubricity, softness and anti-static properties to shaped articles comprising an acrylonitrile polymer containing by weight in the molecule at least 80 percent of acrylonitrile which comprises applying to the article an aqueous dispersion containing from one to 5 percent solids, said solids comprising from 20 percent to 50 percent by weight of sorbitan monopalmitate, from 15 percent to 35 percent of castor oil condensed with from 150 to 250 parts of ethylene oxide, from 10 percent to 40 percent of N-cetyl, N-ethyl morpholinium ethosulfate and from 5 percent to 25 percent of  $\alpha$ ,  $\beta$ -dihydroxyethyl- $\alpha'$ ,  $\beta'$ -di( $\beta$ -stearamidoethyl) urea acetate.

7. A shaped article comprising an acrylonitrile polymer containing at least 80 percent acrylonitrile in the polymer molecule, said article having been treated with a finishing composition comprising an aqueous dispersion having from one to 5 percent solids, said solids comprising from 20 percent to 50 percent by weight of a non-ionic surface active partial ester of a polyhydric alcohol and an aliphatic carboxylic acid, said alcohol having from two to 8 carbon atoms, from 15 percent to 35 percent of a non-ionic surface active polyether prepared by condensing from 150 to 250 parts of ethylene oxide with a member selected from the group consisting of water-insoluble hydroxy-fatty acids, esters of such acids, and mixtures of such acids and esters, and from 10 percent to 40 percent of a cationic surface active quaternary ammonium compound having the formula:



wherein R represents an alkyl radical having less than 5 carbon atoms, R' represents an alkyl radical having less than 5 carbon atoms, and R'' represents an alkyl radical having more than 10 carbon atoms, and from 5

to 25 percent of a substituted carbamyl compound having the formula:



wherein R<sub>1</sub> and R<sub>6</sub> are selected from the group consisting of saturated alkyl radicals containing at least 6 carbons; R<sub>2</sub>, R<sub>3</sub>, R<sub>4</sub>, and R<sub>5</sub> are selected from the group consisting of hydrogen, alkyl, and hydroxyalkyl radicals containing less than 5 carbons and in which R<sub>3</sub> and R<sub>4</sub> may further represent an acid amide chain derived from an acid and a polyamine; D<sub>1</sub> and D<sub>2</sub> are selected from the group consisting of oxygen, sulfur, and imido groups, the number of such groups being as g ranges from 0 to 3; g is an integer from 0 to 3; A is selected from the group consisting of oxygen, sulfur, amino groups, alkyl-substituted amino groups containing less than 5 carbons, and alkylol substituted amino groups containing less than 5 carbons; f and j are integers from 1 to 6; e and k are integers from 0 to 6; m and t are integers from 1 to 6; and X is a negative radical selected from the group consisting of acyl and halogen.

20

25

8. An acrylonitrile polymer in fiber form, said fiber having been treated with an aqueous dispersion containing from one to 5 percent solids, said solids comprising from 20 percent to 50 percent by weight of sorbitan monopalmitate, from 15 percent to 35 percent of castor oil condensed with from 150 to 250 parts of ethylene oxide, from 10 percent to 40 percent of N-cetyl, N-ethyl morpholinium ethosulfate and from 5 percent to 25 percent of  $\alpha$ ,  $\beta$ -dihydroxyethyl- $\alpha'$ , $\beta'$ -di( $\beta$ -stearamidoethyl) urea acetate.

9. An acrylonitrile polymer in fiber form, said fibers having deposited at least on the outer surfaces thereof a conditioning agent comprising a mixture of 20 percent to 50 percent by weight of sorbitan monopalmitate, from 15 percent to 35 percent of castor oil condensed with from 150 to 250 parts of ethylene oxide, from 10 percent to 40 percent of N-cetyl, N-ethyl morpholinium ethosulfate and from 5 percent to 25 percent of  $\alpha$ ,  $\beta$ -dihydroxyethyl- $\alpha'$ , $\beta'$ -di( $\beta$ -stearamidoethyl) urea acetate.

15

#### References Cited in the file of this patent

#### UNITED STATES PATENTS

|           |               |               |
|-----------|---------------|---------------|
| 2,212,369 | Jaeger        | Aug. 20, 1940 |
| 2,293,826 | Iselin et al. | Aug. 25, 1942 |
| 2,304,113 | Morgan et al. | Dec. 8, 1942  |
| 2,686,137 | Rossin et al. | Aug. 10, 1954 |